

Patented June 11, 1929.

1,717,092

# UNITED STATES PATENT OFFICE.

HORACE H. CLARK, OF FARMINGDALE, NEW JERSEY, ASSIGNOR TO CLARK FIBRE PRODUCTS CORPORATION, A CORPORATION OF DELAWARE.

## MOLDED INDURATED-FIBER ARTICLES AND PROCESS OF MAKING SAME.

No Drawing. Application filed January 15, 1927, Serial No. 161,460, and in France June 4, 1926.

This invention relates to the manufacture of boxes, cups or similar articles out of integral masses of cellulose material of the type commonly called "indurated fiber" or "vulcanized fiber".

By these terms is meant a material heretofore usually made out of sheets of paper which, after being separately saturated with a zinc chloride solution, have been placed one 10 on top of another and pressed together in a pile, or rolled up together in a spiral to form a tube which is consolidated by pressure, and finally dried or "cured" after the zinc chloride has been washed out in successive baths 15 of progressively weaker solutions, ending with a washing in fresh water.

So far as I know this material has never been made otherwise than in this "built-up", i. e. originally laminated form. That is to 20 say it has never been possible to make articles (at least not such as have any considerable thickness of walls) by molding a mass of the cellulose pulp directly into the desired final form, and then saturating it with the zinc 25 chloride, or equivalent "indurating" solution, and finally washing and drying it as above described.

The principal reason why this direct molding process has not been followed heretofore 30 has been because the indurating solution (zinc chloride, or its equivalent) has not penetrated more than about fifteen or twenty thousandths (.015 or .020) of an inch below the surface of the dried pulp. Consequently, 35 if the mass to be indurated was more than thirty or forty thousandths (.030 or .040) of an inch thick, there was always left an inner core of fiber never reached by the zinc chloride, and consequently never "indurated", 40 no matter how long the mass was left submerged in the bath. As the material shrinks about 25% in thickness on drying, after treatment with the zinc chloride or other indurating solution as above described, 45 this has heretofore fixed a limit of about thirty thousandths (.030) of an inch for the maximum thickness of wall of any completed article so manufactured, which is little more than the thickness of an egg shell, and too 50 thin for the strength and rigidity usually required.

I have discovered, however, that, by using an improved process in preparing the original pulp from the cellulose fiber, and subjecting the molded blank to compression before

induration, this limit of depth of penetration by the zinc chloride in the "indurating" process can be greatly increased, so that it then becomes possible to mold the pulp into final forms which will have sufficient thickness of 60 wall after "induration" to give them the needed strength. As a result I am able to produce integrally molded articles of indurated fiber having walls of an eighth of an 65 inch and more in thickness, or more than four times the thickness previously possible.

I accomplish this by increasing the capacity of the original dried pulp to uniformly absorb the indurating fluid. The reason (as I believe) why the zinc chloride did not formerly penetrate the dried pulp sheet or blank to a depth of more than about .015 of an inch 70 was traceable to two causes. In the first place, the pulp was not sufficiently freed from gums, and similar impurities of a relatively non-absorbent character, in the usual process of making paper pulp to render it sufficiently hygroscopic. In the second place, an ordinary molded blank of paper pulp has more or less air spaces in its interior. The 75 indurating fluid is so heavy and has such surface tension that after it has penetrated the first few thousandths of an inch from the exterior surfaces of the blank it forms therewith airtight films which hermetically seal the air trapped in the unreached cavities of the remaining, inner portion of the blank's wall, and thereafter the increasing resistance to compression of said trapped air soon 80 checks further inward flow of said indurating solution. I have discovered that if in the original pulp making process the fiber is cooked sufficiently longer, or in a sufficiently 85 increased pressure, the subsequently dried pulp can be rendered so free from such impurities, which are dissolved out by this treatment, that it becomes vastly more hygroscopic and absorbent, and then will much 90 more readily and completely absorb the indurating solution and so allow it to penetrate to greater depths. Also, if the walls of the blank originally molded from such pulp are, before induration, subjected to suitable 95 pressure, as in preliminary forming dies, all air cells therein will be collapsed, and their 100 contained air expelled, so that no trapped air is left to halt the inward progress of the indurating fluid. When this is accomplished, 105 all that remains necessary to produce directly 110

110

molded articles is the devising of molding processes in which such pulp can be conveniently handled, both in the formation of the original molded blank in its compacting 5 prior to induration, and in the final shaping and further compacting of the walls of such blanks.

As an example of the best method at present known to me of carrying out my invention 10 I would proceed as follows:

I preferably take soft cotton rags, such as have been frequently laundered, as the laundering has already removed some of the objectionable gums originally present in the 15 cotton, and turn them into pulp by digesting them in a solution containing about 5 percent of caustic soda (sodium hydrate,  $\text{NaOH}$ ) and about 3 percent of soda (sodium carbonate,  $\text{Na}_2\text{CO}_3 \cdot 10\text{H}_2\text{O}$ ) for about four hours 20 under an atmospheric pressure of from 30 to 50 pounds per square inch. This solution is about 50 percent stronger than that usually employed in making paper pulp. The resultant pulp is consequently of a finer structure, 25 more nearly homogeneous, and contains less gum and similar impurities than does ordinary paper pulp. Consequently it has greater power of absorption. I then mold suitable masses of this pulp into cup-shaped 30 bodies or other forms of dimensions large enough to allow for the ultimate shrinkage that will occur in the drying and indurating steps of the process, by depositing a layer of the pulp preferably on the inside of a per- 35 forated metal former having side walls slightly tapering, like a cone, to a degree such that the cup-shaped mass thus deposited therein can be easily freed therefrom when partially dried. One degree of inclination 40 is sufficient to free a cup two inches deep. A lesser inclination will serve for deeper cups. The walls of these blanks may be partially compacted by pressure in the original mold or former while still wet and then allowed to 45 dry sufficiently to be removed from the former. In some cases they can be shaken out of the mold before drying as the fiber is felted together sufficiently to make them self-sustaining. The blanks are then further 50 dried and subjected to compression in molds to compact the walls and expel the air trapped therein, indurated and finally molded into the desired exact shapes having the desired dimensions in any convenient way.

55 The process of forming or molding the pulp into the original blank may be carried out according to any of the well-known methods, as by pouring as well as by sucking the pulp into a perforated metal former of 60 the desired shape.

The induration of the fiber in the blank may also be carried out in the usual way by immersion in a proper bath of zinc chloride, or the solution described in my pending application Serial No. 697,955, filed March 8,

1924, allowed November 24, 1926, with subsequent washings in progressively weakening baths of the same solution and ultimate washing out in pure water. The impregnated blank may be then, after curing, given 70 its final shape and compactness of wall by compression in any suitable finishing dies.

While the best results are secured by using old cotton rags for making the pulp, a product useful for some purposes may be obtained when other forms of cellulose are substituted.

The main advantage of the invention lies in the successful production of a box, cup or other article having walls of indurated fiber 80 of integral, homogeneous structure, more than .040 inches in thickness, and up to an eighth of an inch and more in thickness, a thing which has not been heretofore in existence, so far as known to me. Boxes and structures 85 for the uses for which the product of my invention is designed have been made usually heretofore of strips of paper and pasteboard glued together. Such gluing cannot be easily done with indurated fiber, and consequently no boxes or similar receptacles of indurated fiber have heretofore been put on the market so far as I know. As indurated fiber 90 is much stronger than pasteboard and capable of receiving more elaborate ornamentation and artistic finish, the advances both in utility and beauty rendered possible by my invention are obvious.

The commercial use of indurated fiber has heretofore been limited to shapes which could 100 be produced by slightly molding sheets, strips or tubes of that material under heat and pressure. The building-up of such laminated sheet or tube, and its subsequent molding under progressive operations by heat and pressure, have been costly and limited in scope.

I am aware that various articles such as 110 pails, bottles, barrels, etc. have been made by flowing paper pulp into molds with perforated walls, and allowing the fiber mass so deposited to dry, but none of these articles was indurated, and the blanks so formed were not further molded after drying, nor were 115 their walls compacted by die pressure, so far as I am aware.

Having described my invention, I claim:

1. The process of making molded integral shapes of indurated fiber which comprises the 120 following steps: Digesting a pulp formed from old cotton cloth in an aqueous solution containing about 5 percent of sodium hydrate and about 3 percent of sodium carbonate for about four hours and under a pressure of from 30 to 50 pounds to the square inch; forming a 125 blank out of said pulp by flowing it into a mold having perforated walls through which is removed a major portion of its water content; drying said blank and impregnating it with an indurating liquid, and finally com- 130

pacting and shaping the walls of said indurated blank by molding under pressure in suitable dies.

2. The process of making molded integral shapes of indurated fiber which comprises the following steps: Digesting a pulp formed from old cotton cloth in an aqueous solution containing about 5 percent of sodium hydrate and about 3 percent of sodium carbonate for 10 about four hours and under a pressure of from 30 to 50 pounds to the square inch; forming a blank out of said pulp by flowing it into a mold having perforated walls through which is removed a major portion of its water 15 content; drying said blank, compacting it by pressure to expel any entrapped air, impregnating it with an indurating liquid, and further compacting and shaping the walls of said indurated blank by molding under pressure 20 in suitable dies.

3. The herein described process which comprises digesting fibrous cellulose in a pulp-making solution of such strength, under such pressure and during such period of time that the resulting pulp, when concentrated, dried 25 and compacted, will form a mass sufficiently hygroscopic to permit an indurating zinc chloride solution to penetrate to a depth of more than twenty thousandths (.020) of an inch from its surfaces; shaping the pulped 30 fiber so obtained in any desired form having walls more than forty thousandths (.040) but not substantially exceeding one eighth of an inch in thickness by depositing it on a foraminous mold, sufficiently compacting the 35 mass under pressure to expel substantially all entrapped air, and impregnating the blank so obtained with a suitable indurating solution, such as one containing zinc chloride.

HORACE H. CLARK.